

1

3,486,838

MODIFICATION OF TEXTILE MATERIAL  
WITH METHYLOLATED LACTAMS

David I. Randall and Harlan B. Freyermuth, Easton, Pa.,  
assignors to GAF Corporation, New York, N.Y., a  
corporation of Delaware  
No Drawing. Filed Oct. 22, 1965. Ser. No. 502,387  
Int. Cl. D06m 13/02

U.S. CL. 8—115.5

8 Claims

ABSTRACT OF THE DISCLOSURE

Reaction of fibrous materials containing labile hydrogen atoms and heterogeneous blends thereof with N-methyloxylactams or the lower alkyl ether derivatives thereof in the presence of an acid catalyst at elevated temperatures. Fibrous material dye affinity is modified.

The present invention relates to a method for treating fibrous materials in order to improve the properties thereof and to the improved fibrous materials produced thereby. More particularly, the present invention relates to a method for improving the receptivity of fibrous materials, preferably of the cellulosic variety, including blends thereof with other fibrous materials of the natural and/or synthetic types, to dyestuffs and fluorescent brightening agents not ordinarily substantive thereto. This invention also relates to an improvement in such other properties of fibrous materials as resistance to attack by mildew, laundry sours and the like, and to shrinking, washing and the like.

As is well known, fibrous materials consisting in whole or in part of cellulosic materials such as cotton and the like in general possess poor receptivity for a considerable number of the commercially available dyestuffs commonly employed in fiber coloring operations. For example, many of the dyestuffs which can be effectively employed with natural and synthetic fibers such as wool, nylon, etc., possess little or no affinity for cellulosic materials, at least to the extent of satisfying the requirements of commerce. Certain fiber-pretreatment methods have heretofore been proposed by which the physical and/or chemical characteristics of cellulosic fibrous material are altered to thereby produce a fibrous material allegedly characterized by improved receptivity to dyestuffs not ordinarily substantive thereto. For example, it has been previously suggested to treat fibrous materials at any stage of the coloring operation, i.e., before, during or after the dyeing step with polymerizable monomeric materials which are thereafter made to undergo polymerization in situ on and/or with the fibrous material, or alternatively, to treat the fibrous material directly with the resin in solution form. However, such methods suffer from several disadvantages among the more notable being the high cost of resin and resin-forming materials and the tendency of such materials to undesirably affect the character and properties of fibrous materials treated therewith. It has also been suggested, as a method of improving dye receptivity, to pretreat cellulosic fibrous materials with a compound which is reactive therewith. However, fiber-treating methods based on the use of the "reactive compounds" thus far proposed, though enhancing somewhat the properties of fibrous materials treated therewith, leave much to be desired with respect to such desirable properties in the resultant fiber as receptivity to dyestuffs, fluorescent brightening agents and the like as well as resistance to attack by mildew, laundry sours and the like.

Accordingly, it is an object of this invention to provide a method for improving the properties of fibrous

2

materials which will not be subject to one or more of the above disadvantages.

Another object of this invention resides in the provision of fibrous materials having improved properties. Still other objects and advantages of the invention will become further apparent from the following detailed description thereof.

In accordance with the aforesaid objects of the invention, methods have been devised for the achievement thereof which comprise treating a fibrous material with an aqueous solution containing at least one lactam compound selected from the group consisting of compounds of the formula:



20 and ring carbon-lower alkyl substituted derivatives thereof, wherein R represents an alkylene bridge such as, for example, ethylene, propylene, butylene, necessary to complete a 5 to 7 membered heterocyclic ring; and R' represents hydrogen or lower alkyl such as methyl, ethyl, propyl and the like; and subsequently drying and curing the treated material at a temperature of at least about 120° C. The invention also comprises the provision of fibrous materials having improved receptivity to dyestuffs which ordinarily display but negligible affinity for cellulosic fibrous materials such as those employed in coloring wool, nylon and the like. Moreover, it has been found that when fibrous materials are treated according to the present invention there is obtained a fiber product which exhibits, in addition to the improved properties of the above-described type, surprisingly good receptivity to fluorescent brightening agents.

This result is particularly significant since many of the synthetic fibers and their blends with cellulosic materials as typified, for example, by nylon-cotton, Dacron-cotton, acrylic-cotton and the like, have proved relatively difficult to whiten to the desired extent.

40 A preferred class of compounds for use in the present invention, particularly for improving the receptivity of fiber materials to dyestuffs and fluorescent whiteners, is the class of compounds of the above formula wherein R represents the carbon atoms necessary to complete a 2-pyrrolidone ring, i.e., R in the above formula is ethylene. These compounds can be structurally depicted as follows:



50 and the ring carbon-lower alkyl substituted derivatives thereof, where R' is hydrogen or lower alkyl. These compounds can be easily and conveniently prepared in known manner from the parent pyrrolidone. The compound of the above formula wherein R' is hydrogen, i.e., N-hydroxymethylpyrrolidone, is formed by reacting 2-pyrrolidone with paraformaldehyde in the presence of an alkaline catalyst such as potassium hydroxide. Compounds of the above formula where R' is lower alkyl can be formed by reacting 2-pyrrolidone with a mixture of paraformaldehyde and an alcohol.

55 The compounds of Formula I above wherein R' represents the carbon atoms necessary to complete either a 2-piperidone or -caprolactam ring, i.e., R' is propylene or butylene, respectively, are also highly effective agents for increasing the dye and fluorescent brightener recep-

tivity of fibrous materials treated therewith. The compounds can be structurally depicted as follows:



as well as the ring carbon-lower alkyl substituted derivatives thereof, wherein R' is hydrogen or lower alkyl. Compounds of the above formulae can be prepared by N-methylation or N-alkoxymethylation of the parent piperidone-2 and -caprolactam compounds in the same manner as described in connection with the preparation of the compounds of Formula II hereinabove.

The process of the present invention is applicable in general to fibrous materials constituted in whole or in part by labile hydrogen-containing substances such as cotton and other materials of the cellulosic type. As illustrative of the foregoing class of materials there may be mentioned textiles comprising 100 percent cotton, linen and the like and blends of fibers of cellulosic materials with fibers of other materials such as regenerated cellulose, e.g., viscose rayon or cuprammonium rayon, polyamides such as nylon, e.g., the polyamide of hexamethylene diamine and adipic acid or of 6-aminocaproic acid; polyurethanes; acrylonitrile polymers and copolymers; polyesters such as polyethylene terephthalate; animal fibers such as wool and mohair; cellulose esters, e.g., cellulose acetate, cellulose propionate, cellulose butyrate, cellulose acetate-propionate, cellulose acetate-butyrate and the like and cellulose ethers such as ethyl or benzyl cellulose.

In carrying out the method of the present invention according to the preferred manner, an aqueous medium containing at least one lactam derivative of the type depicted in the foregoing formulae is applied to the fibrous material, following which the material so treated is dried and cured. The aqueous medium may be in the form of a solution, emulsion, suspension or other type of dispersion depending for example upon the physical properties of the particular lactam derivative employed. Although the lactam derivatives of the present invention are all readily water soluble or dispersible, it may in some instances be desired to promote lactam solubility as for example by moderate heating of the aqueous media. Moreover, the aqueous medium may further contain any suitable stabilizer, surface active agent and the like to assist in providing a suitably uniform medium for the fiber treatment. The aqueous medium may in addition contain a swelling agent for the fibrous material such as, for example, the butyl ether of ethylene glycol, acetone, dioxane and the like to promote conformity of distribution of the lactam derivative throughout the fibrous material.

Preferably, the aqueous treating medium is further provided with an acid catalyst. Suitable catalysts are those which are acidic at the temperatures employed when applying the lactam solution to the fibrous material. As representative catalyst materials these may be mentioned by way of illustration—ammonium phosphate, also known as "accelerator 187," zinc chloride and zinc nitrate and the like. Acid-bound alkanol amines such as 2-methyl-2-amino-1-propanol hydrochloride, also known as "catalyst AC" are particularly effective catalysts for carrying out the present invention. Other suitable catalysts are ammonium sulfate, oxalic acid and the amine hydrochloride known as "Aerotex Accelerator 187" and the like. The catalyst may advantageously be added to the aqueous treating medium in the form of an aqueous solution just before the mixture is applied to the textile material. Catalyst proportions are not particularly critical and may range from about .1 percent to 15 percent and higher based on the weight of lactam. However, in certain instances, the amount of catalyst should be increased. For example, if an alkaline substance is present in the

fibrous material, e.g., as an impurity, it will probably "poison" the catalyst by reacting therewith, thereby reducing the effective amount of catalyst available for the fiber treatment. Accordingly, in such a case, the amount of catalyst should be increased to provide the desired effective amount thereof.

The concentration of the lactam derivative in the aqueous medium is not particularly critical and may range from about 0.5 to 50 percent and higher, depending for example upon the method employed for applying the medium to the fibrous material, the particular lactam derivative and fibrous material employed, the properties desired in the fibrous material, etc. The aqueous treating compositions may be applied to the fibrous material by immersion, padding, spraying, painting or any other desired manner, continuous or otherwise. When overall effects are desired in the fabric material, it is preferred to apply an excess of the aqueous treating composition thereto followed by removal of excess as by squeezing, spinning, etc.

Following application of the aqueous solution of lactam derivative, the fibrous material is dried and then cured at a temperature of at least about 120° C. The drying can be effected at temperatures of up to about 95° C. and higher, depending merely on the rate of drying desired. The duration of the curing step will in general vary inversely with the temperature employed although, of course, the temperature and time factors will also depend somewhat upon the type of fibrous material being treated, the particular lactam treating agent employed, the results desired, etc. In any event, the optimum curing parameters of time and/or temperature, may, in any particular instance, be readily determined by routine experimentation. For example, as a general indication of the effect of the time temperature parameters on curing, it can be expected that the curing time will usually range up to five minutes or more for temperatures in the vicinity of approximately 150° C.-155° C. with cotton materials, while the use of higher temperatures, e.g., up to 250° C. and higher, reduce proportionately the curing time required to—in some instances—a matter of seconds. Following the curing operation, the fibrous material is desirably washed, preferably in the presence of a mild detergent, to remove any residual acidity, etc., and prevent the development of odor.

The mechanism by which the process and compositions of the present invention yield fibrous materials having improved properties of the type enumerated hereinabove is not completely understood but can be postulated as follows. Apparently, the labile hydrogen atoms present in the molecular structure of the fibrous material being treated enter into reaction with the N-methylol or N-alkoxymethyl substituent of the lactam derivative. Apparently an initial hydrolysis reaction occurs with the N-alkoxymethyl derivatives whereby such groups are converted to methylol. The labile hydrogen of the fibrous material may be present in the form of hydroxy, carboxy, amido, amino and/or cyano (hydrolysis provides amido and carboxyl hydrogen) and the like.

For example, the hydroxy groups may be present in the form of alkylol, e.g., methylol such as found in cellulose, its partial ethers and esters and cellulosic type materials such as cotton, or as glycol residues containing free hydroxy such as found in synthetic polyesters of the linear variety or such groups in vinyl type synthetic polymers. Illustrative of the materials which contain and/or provide labile hydrogen in the form of carboxy are the synthetic vinyl-type polymers known as the "acrylics," synthetic polymers of the polyester type containing free carboxy within the molecular structure thereof, and materials which contain functional groups convertible to carboxy under the conditions of the treatment process described herein such as wool and polymers from acrylonitrile and the like. Illustrative of the materials which contain and/or provide labile hydrogen in the form of amino and amido under the conditions of the treatment process described

herein are vinyl type polymers containing recurring amino or amido side groups such as polyvinylamines, polyacrylamide, etc., wool, nylon, hydrolyzed acrylonitrile polymers, etc. In any event, it is quite apparent that the lactam derivatives of the present invention chemically combine with the fibrous material being treated as evidenced by chemical analysis of the treated fiber product, application of severe wash tests, etc., as will be apparent from the examples given hereinbelow.

As stated hereinabove, the process of this invention is found to be highly effective for improving the properties of fibrous materials containing labile hydrogen within the molecular structure thereof, e.g., cellulosic materials such as cotton and the like, synthetic and animal fibers of the type indicated hereinabove, and blends of two or more of the foregoing materials. The fibrous material may be in any of the usual forms, e.g., staple, fiber or continuous filament in bulk form or in the form of tow, rope, yarns, slubbings, warps, fabrics, felts, and the like, and treated as a wound package, running length fibrous stock, bulk, etc.

The fibrous materials obtained by the process of the present invention exhibit a pronounced "animalization" effect which is probably due to the presence therein of chemically bound nitrogen, e.g., in the form of amide groups, resulting from the chemical interaction of the fibrous material and lactam derivative. Accordingly, the resultant fibrous material is characterized by many "wool-like" properties, such as a pronounced receptivity for acid dyes, basic dyes, wool dyes, etc., fluorescent brighteners and the like.

The following examples are given only for purposes of illustrating the present invention and are not to be regarded as limitative thereof. All parts and proportions referred to herein and in the appended claims are by weight unless otherwise indicated.

#### EXAMPLE 1

An aqueous solution containing 10 parts of N-hydroxymethylpyrrolidone and 0.36 part of the catalyst 2-methyl-2-amino-1-propanol hydrochloride, which is added in the form of a 25 percent aqueous solution thereof, is applied by padding to cotton print cloth, 80 x 80, at room temperature. The treated cloth is squeezed through rubber rollers to 100 percent weight pickup of solution and thereafter dried at about 80° C.-85° C. The dried cloth is thereafter heat aired at 150° C.-155° C. for approximately 3 minutes. Following this, the fabric is rinsed with cold water, boiled for approximately 10 minutes in the presence of a small amount of non-ionic detergent and rinsed again in cold water. Chemical analysis (Kjeldahl method) of the treated cloth indicates that approximately 83 percent of the N-hydroxymethylpyrrolidone-2, over and above that lost by sublimation (approximately 36 percent), is introduced into the treated cloth.

#### EXAMPLE 2

Example 1 is repeated except that the cotton print cloth is replaced by a sample of Dacron-cotton (60/40) fabric. Results similar to those of Example 1 are obtained.

The fibrous materials obtained from Examples 1 and 2 are found to possess in comparison to untreated control samples of the foregoing fibrous materials, significantly improved receptivity for basic dyes, acid dyes, wool dyes, etc., which are conventionally employed in dyeing wool, nylon and the like and which possess little or no affinity for untreated cellulose materials. Further surprising is the discovery that the fibrous materials provided by the foregoing examples display, in addition to the above mentioned properties, a pronounced affinity for fluorescent brightening agents commonly employed with wool, nylon, etc., as compared to untreated control samples of such fibrous materials.

The following examples illustrate the improved receptivity of fibrous materials which have been treated in ac-

cordance with the present invention to the above-mentioned dyestuffs and fluorescent brightening agents.

#### EXAMPLE 3

The cotton print cloth obtained from Example 1 and the Dacron-cotton (60/40) material obtained from Example 2 are each treated separately with an amino-coumarin fluorescent brightening agent of the following formula:



The above compound is found to be substantive to each of the cloth samples which display a pronounced fluorescent brightness in comparison to untreated control samples of each of these fibrous materials.

As further illustrative of fluorescent brightening agents which may be used with fibrous materials treated according to the present invention with the intention of like results there may be mentioned by way of example the amino coumarins described in U.S. Patent 2,610,152, the 4,4' - di - trizyldiaminostilbene - 2,2' - disulfonic acid derivatives described in U.S. Patent 2,612,501; the bis(2-morpholino - 4 - amino - 1,3,5 - triazyl - (6) - ) 4,4' - diaminostilbene sulfonic and carboxylic acid materials described in U.S. Patent 2,618,636; the hydroxybenzimidido-azolylstilbene carboxy esters described in U.S. Patent 2,937,997; the 4,5-diphenyl glyoxalone-disulfonic acid derivatives described in U.S. Patent 2,691,653; and the brightening agents described in U.S. Patent 2,688,777.

#### EXAMPLE 4

Samples of cotton print cloth, 80 x 80, and Dacron-cotton, 60/40) treated according to the process described in Example 1 are dyed at the boil with a 1 percent aqueous solution of the acid dyestuff Colour Index Acid Yellow 121; C.I. No. 18690. The foregoing dyestuff exhibits a pronounced affinity for each of the cloth samples treated therewith which exhibit a vivid overall yellow color. Control samples of the untreated cloth materials exhibit negligible receptivity for the same dyestuff.

A similar improvement in receptivity to acid dyes, basic dyes, wool dyes, etc., is obtained when samples of cotton print cloth and Dacron-cotton (60-40), each treated in accordance with Example 1, are separately dyed at the boil with aqueous solutions (1 percent) of the following dyestuffs.

##### Colour Index—

|    |                                 |
|----|---------------------------------|
| 55 | Acid Red 182                    |
|    | Acid Blue 179                   |
|    | Acid Black 107                  |
|    | Acid Orange 60                  |
|    | Acid Red 273                    |
| 60 | Acid Red 114; C.I. No. 23635    |
|    | Acid Blue 62; C.I. No. 62045    |
|    | Acid Green 25; C.I. No. 61570   |
|    | Acid Black 48; C.I. No. 65005   |
|    | Acid Orange 72; C.I. No. 18740  |
| 65 | Acid Red 183; C.I. No. 18800    |
|    | Acid Black 52; I.I. No. 15711   |
|    | Basic Red 14                    |
|    | Basic Red 13; C.I. No. 48015    |
|    | Basic Red 15                    |
|    | Basic Blue 5; C.I. No. 42140    |
| 70 | Basic Orange 22; C.I. No. 48040 |

In each case, the samples of treated cloth exhibit a pronounced receptivity for each of the above dyestuff materials in comparison to control samples of untreated cloth which exhibit but negligible receptivity therefor.

As stated previously, although the above dyestuff products are commonly used in coloring fibrous materials comprising wool, nylon, acrylic materials and the like, they ordinarily display but negligible affinity for untreated fibrous materials consisting in whole or in part of cellulosic substances. However, by the process of the present invention, there are provided improved fibrous materials which are characterized by a pronounced affinity for such acid, wool, and basic dyestuffs and the like, as well as a pronounced affinity for fluorescent brightening agents such as of the type hereinbefore indicated.

Furthermore, similar improved results as regards dye and fluorescent brightener receptivity are obtained when the procedure of Example 1 is repeated utilizing similar weight proportions of catalyst and lactam material but wherein the following compounds are substituted for the N-hydroxymethylpyrrolidone-2 compound of Example 1.

Pyrrolidones

N-methoxymethyl pyrrolidone-2  
3,3-dimethyl-N-hydroxymethylpyrrolidone-2  
3,3,5-trimethyl-N-hydroxymethylpyrrolidone-2  
3,3,5-trimethyl-N-methoxymethylpyrrolidone-2  
3-propyl, 5-methyl-N-hydroxymethylpyrrolidone-2

Piperidones

N-hydroxymethylpiperidone-2  
N-methoxymethylpiperidone-2  
4,4-dimethyl-N-hydroxymethylpiperidone-2  
6-propyl-N-methoxymethylpiperidone-2  
4,4-dimethyl-N-ethoxymethylpiperidone-2

Epsilon-caprolactams

3,3,5-trimethyl-N-hydroxymethyl-E-caprolactam  
N-hydroxymethyl-E-caprolactam  
N-methoxymethyl-E-caprolactam  
4,4-dimethyl-N-ethoxymethyl-E-caprolactam

In each case, the samples of cotton print cloth and Dacron-cotton (60-40) obtained with the above compounds according to the process of Example 1 exhibit pronounced affinity for the dyestuffs and fluorescent brightening agents of the type enumerated hereinabove.

As previously pointed out, the fibrous materials provided by the process of the present invention are additionally characterized by an improvement in such other properties, such as resistance to attack by mildew as will be apparent from the following example:

EXAMPLE 5

Samples of cotton print cloth, 80 x 80 and Dacron-cotton (60/40) each treated in accordance with the process of Example 1 are subjected, along with untreated control samples of the foregoing materials, to soil burial tests for a period of approximately two weeks. In each case, the treated cloth samples exhibited improved resistance to mildew as compared to the untreated samples.

It has also been found that the cellulosic materials treated in accordance with the present invention are capable of complexing or compounding with a variety of germicidal agents such as iodine and reducing the vapor

pressure of the germicidal agent so that it remains on the cloth for substantial periods of time. The combination of iodine and other germicidal and disinfecting agents with cloth treated in accordance with the present invention to produce germicidal bandages, surgical dressings, and the like, forms the subject matter of the copending application of Leon Katz, filed Oct. 22, 1965, Ser. No. 502,618, now Patent 3,401,005 which most fully describes and claims the same.

While the invention has been described in particularity with respect to certain embodiments thereof, it will be obvious to those skilled in the art that numerous modifications and variations of the invention can be made without departing from the spirit and scope thereof. Therefore, it is intended that in the claims which follow the invention be interpreted as inclusive of all such modifications and variations insofar as the state of the art permits.

What is claimed is:

1. A process comprising treating fibrous materials containing labile hydrogen atoms with a composition consisting essentially of a compound selected from the group consisting of lactam derivatives of the formula:



30 and ring carbon-lower alkyl substituted derivatives thereof, and wherein R represents a lower alkylene group necessary to complete a 5 to 7 membered heterocycle and R' is selected from the group consisting of hydrogen and lower alkyl, and an acid catalyst contained in an aqueous medium, then drying and curing the fibrous material at a temperature of at least about 120° C.

2. A process as defined in claim 1 wherein the fibrous material contains a cellulosic material.

3. A process as defined in claim 1 wherein the lactam derivative is N-hydroxymethylpyrrolidone-2.

4. A process as defined in claim 1 wherein the lactam derivative is N-hydroxymethylpiperidone-2.

5. A process as defined in claim 1 wherein the lactam derivative is N-hydroxymethyl-caprolactam.

6. A process as defined in claim 1 wherein the lactam derivative is N-methoxymethylpyrrolidone-2.

7. A process according to claim 1 wherein the acid catalyst is 2-methyl-2-amino-1-propanolhydrochloride.

8. A fibrous material produced according to the process of claim 1.

References Cited

UNITED STATES PATENTS

1,070,588 12/1959 Germany.

55 GEORGE F. LESMES, Primary Examiner

J. CANNON, Assistant Examiner

U.S. CL. X.R.

60 8—31, 55, 57, 100, 115.7, 116.2, 116.3, 127.6, 129